

# UNITED STATES PATENT OFFICE.

DONATO DI CARLO, OF PHILADELPHIA, PENNSYLVANIA.

## DIAPHRAGM FOR SOUND-BOXES.

1,330,060.

Specification of Letters Patent. Patented Feb. 10, 1920.

No Drawing.

Application filed February 26, 1919. Serial No. 279,391.

To all whom it may concern:

Be it known that I, DONATI DI CARLO, a subject of the King of Italy, having declared my intention of becoming a citizen of the United States, and a resident of Philadelphia, county of Philadelphia, State of Pennsylvania, have invented Diaphragms for Sound-Boxes, of which the following is a specification.

10 My invention relates to diaphragms for use in connection with sound reproducing instruments, as, for instance, in the sound box of a talking machine; the object of my invention being the formation of a diaphragm combining improved sound transmitting qualities with strength and durability and with an extremely low production cost.

20 In general, the diaphragm consists of a base of mineral material possessing the characteristics of cement, such as china clay or plaster of Paris, to which is added an amount of a metallic oxid or oxids, preferably oxid of zinc, these materials being incorporated 25 with a mucilaginous binder such as shellac or glue. In forming the diaphragm I have obtained the best results by subjecting the mixture to heat until the mass is thoroughly incorporated, after which it is poured into 30 molds of the desired shape and size and allowed to cool and to set. This diaphragm disk I have found to possess greatly improved sound transmitting qualities, is strong and durable, and the cost of the raw 35 materials and of production are very low.

As a specific example of my invention, I may form a mixture of plaster of Paris, 40 oxid of zinc, and white glue, and water, these substances forming approximately 50%, 10% 30% and 10% respectively of the total volume of the mass. Heat is now applied to this mixture until the glue is dissolved and the mass thoroughly incorporated, after which it is poured into molds 45 and allowed to cool. The addition of a small amount of lamp black will make the material black if this is desired, without otherwise affecting the finished product.

As previously stated, various metallic oxids may be employed, though I believe 50 the oxid of zinc gives the best results, and this oxid is therefore preferred. When gum shellac is employed as the binder, a nitrohydrocarbon, or suitable solvent material for the shellac, must also be used, 55 such solvent material not acting to alter the characteristics of the finished diaphragm. Lamp black may be employed to blacken the diaphragm material if desired.

It will be evident that there exists a wide 60 latitude in the use of materials and in their relative proportions, and it will be understood that I do not wish to be limited to any set formula, nor to any fixed method of forming the diaphragm. But what I claim 65 as my invention and desire protection upon is:—

1. A diaphragm for sound reproducing apparatus comprising a cementitious mineral base, a metallic oxid, and a mucilaginous binder. 70

2. A diaphragm for sound reproducing apparatus comprising a base of plaster of Paris, a metallic oxid, and a mucilaginous binder. 75

3. A diaphragm for sound reproducing apparatus comprising a base of plaster of Paris, oxid of zinc, and a mucilaginous binder. 80

4. A diaphragm for sound reproducing apparatus comprising plaster of Paris, oxid of zinc, and glue, the ratio of the volumes of such comprised substances being approximately 50 to 10 to 30 respectively. 85

5. The process of forming a diaphragm 90 for sound reproducing apparatus comprising intimately mixing 50 parts by volume of plaster of Paris with 10 parts of oxid of zinc and 30 parts of glue, adding approximately 10 parts of water, applying heat to 95 said mixture until the glue is dissolved and the mass thoroughly incorporated, and pouring said incorporated mixture into molds and allowing it to cool therein.

DONATO DI CARLO.